

June 14, 1949.

F. H. BRITTAI N ET AL

2,472,938

POINT-CONTACT RECTIFIER

Filed March 1, 1945



INVENTORS  
FRANCIS H. BRITTAI N AND  
CHARLES E. RANSLEY

BY

*John A. Harvey*

ATTORNEY

## UNITED STATES PATENT OFFICE

2,472,938

## POINT-CONTACT RECTIFIER

Francis Hugh Brittain, Pinner, and Charles Eric Ransley, Sudbury, England, assignors to The General Electric Company Limited, London, England

Application March 1, 1945, Serial No. 580,484  
In Great Britain November 8, 1943

Section 1, Public Law 690, August 8, 1946  
Patent expires November 8, 1963

10 Claims. (Cl. 175—366)

1

This invention relates to point contact rectifiers that is to say combinations of a semi-conducting crystal (usually nowadays consisting mainly of silicon often with small additions of aluminium or beryllium or both) and a metal wire (usually of tungsten) whose pointed end rests on the crystal. The pointed end may be shaped to give contact substantially at a point or along a line. The terms "point contact" or "pointed end" are intended to cover both forms. The invention relates also to their manufacture.

When such rectifiers are used at frequencies of the order of 10,000 mc./s., the capacitance of the contact is of great importance; it should be as small as possible. The object of this invention is to reduce this capacitance.

We have found that an increase of the hardness of the pointed end of the wire may lead to a decrease of the smallest attainable capacitance, and that the hardness of the usual tungsten point may be conveniently increased for this purpose by carbonising it in known manner. The reason for this decrease in capacitance is due to a lessening of the deformation of the tungsten point, the hardening of the tungsten point rendering it more resistant to such deformation.

According to one aspect of the invention, the manufacture of a point contact rectifier comprises the step of subjecting the said pointed end to a hardening treatment.

According to another aspect of the invention, in a point contact rectifier the said wire is of tungsten and its pointed end is carbonised. The single figure of the drawing illustrates a suitable construction for a point contact rectifier of the type herein described.

The wire usually has a bent portion that provides the elasticity necessary in order that the pressure of the point on the crystal may be regulated. This part is preferably not hardened. Again when the point has been hardened it is liable to penetrate the surface layer of the crystal on whose presence efficient rectification depends. The tendency to penetrate may be decreased by subjecting the point to electrolytic etching of known kind; the effect of the etching is probably to smooth the surface of the point.

In one method of manufacture according to the invention, the wire is of tungsten 0.2 mm. in diameter with the end sheared off at an angle of about 45° to the axis of the wire to form a pointed end. The necessary elasticity is provided in known manner, by an S-bend a short distance from the pointed end. The pointed end is carbonised and the bent portion is excluded

2

from such carbonising by bringing the pointed end into contact for a few seconds with a carbon block heated to 1500–1600° C. in a non-oxidising atmosphere. The pointed end is then etched for a few seconds by the use of alternating current and an alkaline solution.

In another method of manufacture according to the invention, the wire is again of tungsten, its pointed end is shaped, and the wire is provided with an S-bend, as in the previous example. The local carbonising of the pointed end, whilst excluding the bent portion from such carbonising, is achieved by introducing the wire into a bell jar in which is a stout filament of suitable material such as tungsten, heated to a temperature of 1500–2000° C. The said pointed end is brought to touch the stout tungsten wire for a few seconds whilst an atmosphere containing hydrocarbon vapour is passed through the bell jar.

20 A suitable atmosphere is 80% nitrogen, 20% hydrogen, saturated with xylene vapour. The saturation may be produced by bubbling the nitrogen and hydrogen mixture through the hydrocarbon at room temperature. The pointed end is then etched as in the previous example.

A suitable co-operating crystal is one of the kind described in United States Letters Patent No. 2,419,561, granted April 29, 1947, to Jones et al. The rectifier may be completed in any known or suitable manner by mounting the point contact in such a manner that its pointed end bears with a suitable pressure upon a surface of the crystal. For example, and referring to the single figure of the drawing, a point contact rectifier may conveniently be constructed by the use of a hollow cylindrical ceramic body member 10 having conductive terminals 11, 12 threaded into individual ends thereof. The pointed metal wire 13 includes an unhardened S-bend as heretofore mentioned and is soldered at its blunt end into a coaxial bore 14 of the terminal 12. The semi-conducting crystal 15 is soldered on the end of a conductive pin 16 which is adjustably positioned in an axial bore 17 of the terminal 11 and is retained in adjusted position therein by a set screw 18 threaded through the side of the terminal 11. During assembly of the rectifier, the pin 16 is pushed through the bore 17 of the terminal 11 until the semi-conducting crystal 15 engages the hardened point of the wire 13 and slightly compresses the latter. The pin 16 may thereafter be slightly rotated to position the pointed metal wire 13 on a sensitive spot on the surface of the semi-conducting crystal 15 after which the set screw 18 is set to maintain the pin 16 in its ad-

justed position. The ceramic body 10 is provided with an aperture 19 by which the cavity within the body may conveniently be filled with a wax to maintain the metal wire 13 in adjusted position on the semi-conducting crystal 15 and also to render the point contact rectifier moisture proof.

It has been found possible with the aid of the present invention to achieve readily capacities of the order of 0.05-0.10 micro-microfarads. With 10 previously known methods the capacity is 0.25-0.5 micro-microfarads or even greater.

We claim:

1. A method of manufacturing a point contact rectifier comprising a semi-conducting crystal and a metal wire whose pointed end rests upon said crystal which comprises the step of subjecting said pointed end to a hardening treatment.

2. A method according to claim 1, wherein said metal wire has a bent portion to provide the elasticity necessary in order that the pressure of the point on the crystal may be regulated, and wherein said bent portion is excluded from said hardening treatment.

3. A point contact rectifier comprising a semi-conducting crystal and a metal wire whose pointed end rests upon said crystal, wherein said metal wire is of tungsten and the pointed end thereof is carbonised.

4. A point contact rectifier comprising a semi-conducting crystal and a metal wire whose point end rests upon said crystal, wherein said metal wire has a bent portion to provide the elasticity necessary in order that the pressure of the point on the crystal may be regulated and wherein in the pointed end of said wire is harder than said bent portion.

5. A point contact rectifier according to claim 3, wherein said hardened, pointed end has an 40 etched surface.

6. A method of manufacturing a point-contact rectifier comprising a semi-conducting crystal and a tungsten wire having a pointed end resting upon said crystal which comprises the step of hardening said pointed end of said tungsten wire by subjecting said pointed end to a carbonising treatment.

7. A method of manufacturing a point-contact rectifier comprising a semi-conducting crystal and a tungsten wire having a pointed end resting upon said crystal which comprises the step of hardening said pointed end of said tungsten wire by bringing said pointed end into contact with carbon heated to a suitable high temperature in a non-oxidising atmosphere.

8. A method of manufacturing a point-contact rectifier comprising a semi-conducting crystal and a tungsten wire having a pointed end resting upon said crystal which comprises the step of hardening said pointed end of said tungsten wire by heating said pointed end to a suitable temperature in an atmosphere containing a hydrocarbon vapour.

9. A method of manufacturing a point-contact rectifier comprising a semi-conducting crystal and a tungsten wire having a pointed end resting upon said crystal which comprises the step of hardening said pointed end of said tungsten wire by heating said pointed end to a suitable high temperature in an atmosphere containing a hydrocarbon vapour, said heating of said pointed end being effected by bringing said pointed end into contact with a heated tungsten wire.

10. A method of manufacturing a point-contact rectifier comprising a semi-conducting crystal and a metal wire having a pointed end resting upon said crystal which comprises the steps of subjecting said pointed end to a hardening treatment, and subsequently subjecting said hardened pointed end to electrolytic etching in order to reduce the tendency of said hardened pointed end to penetrate the surface layer of said crystal.

FRANCIS HUGH BRITTAINE.  
CHARLES ERIC RANSLEY.

#### REFERENCES CITED

The following references are of record in the file of this patent:

#### UNITED STATES PATENTS

| Number    | Name            | Date          |
|-----------|-----------------|---------------|
| 1,611,653 | Lilianfeld      | Dec. 21, 1926 |
| 1,708,572 | Hartmann et al. | Apr. 9, 1929  |